

## UNITED STATES PATENT OFFICE.

JOSEPH ALEXANDER YOUNG, OF BELLEVUE, PENNSYLVANIA.

## OIL COMPOSITION.

No Drawing.

Application filed May 6, 1922. Serial No. 559,058.

*To all whom it may concern:*

Be it known that I, JOSEPH A. YOUNG, a citizen of the United States, residing at Ben Avon Heights, Bellevue, county of Allegheny, and State of Pennsylvania, have invented certain new and useful Improvements in Oil Compositions; and I do hereby declare the following to be a full, clear, and exact description of the invention, such as 10 will enable others skilled in the art to which it appertains to make and use the same.

This invention relates to oil compositions; and it relates more particularly to an oil composition comprising a mineral oil base 15 in which is dissolved camphor, said composition being of special utility for lubricating leaf springs on motor vehicles, for loosening nuts, machine screws, or the like, that have become rusted or otherwise fixed 20 in place, and for other analogous purposes.

In general, the oil constituting the base of my novel oil composition should be mineral oil; and most desirably there should be no animal or vegetable oil in the composition. Dissolved in the mineral oil base is a 25 quantity of camphor, ordinary commercial gum camphor being suitable and being employed in proportion which may vary but which is ordinarily small. The complete oil 30 composition should be penetrating in character so that it may readily enter extremely small cracks and crevices, but it should nevertheless embody good lubricating properties. The camphor contributes toward the 35 penetrative characteristic; also it acts as a rust-cutting agent and rust deterrent, the term rust being here used broadly to designate any form of corrosion or the like that causes contacting parts to become locked or 40 "frozen" together. The mineral oil base may vary considerably in its specific character so long as it provides, in combination with the admixed camphor, a highly penetrating oil composition, carrying lubricating 45 values and possessing rust-cutting and protective properties as hereinabove set forth.

By way of a concrete example embodying the principles of the invention, reference 50 may be made to one specific form of my novel composition which has proved especially effective in use and which constitutes the best mode now known to me of practicing the invention. In this particular instance, the mineral oil base consists of a mixture of good quality lubricating oil, such as

a medium motor oil, and a high grade Pennsylvania crude petroleum; and with this base is incorporated the desired amount of commercial gum camphor. The ingredients may advantageously be compounded in the 60 approximate proportions of 4 parts of said lubricating oil, 11½ parts of the crude petroleum, and ½ part camphor, all parts being by weight. Although these proportions are especially desirable and are recommended 65 as best, they may be varied considerably while still realizing the benefits of the invention to a substantial extent. A convenient way of incorporating the camphor with the oil is to dissolve it in a part of the crude oil 70 with the aid of heat, and then to mix the solution with the rest of the oil. This is merely typical, however, of procedures that may be followed. The use of heat is not essential although it expedites the operation of 75 compounding the mixture. In general, the proportion of camphor need not exceed 2 ounces per pint of the finished composition, and a substantially smaller proportion is ordinarily preferable.

In the specific example above given, the lubricating oil employed tested as follows: Baumé gravity 28.7; viscosity at 100° F., 300; flash, 435° F.; fire, 485° F.; pour test, 20° F.; demulsibility, 172; conradson 80 carbon, .25%; acid number, .09 equal to .05% oleic.

The crude petroleum tested as follows: Baumé gravity, 47.0.; distillation, initial boiling point, 50° C.; 10% over at 113° C.; 90 20% over at 143° C.; 30% over at 170° C.; 40% over at 210° C.; 43% over at 220° C. (yield of gasoline); 50% over at 247° C.; 60% over at 288° C.; 63% over at 300° C. (yield of kerosene).

The use of a crude petroleum in the mixture is advantageous because it carries not only a certain proportion of lubricating oil fractions but also lighter fractions, such as the gasoline and kerosene fractions, that contribute toward the penetrating character of the final composition.

The complete finished composition obtained in the above specific example is thinly fluid and highly penetrating, shows a typical mineral oil bloom, and smells strongly of camphor.

It is to be understood that the foregoing specific examples of oils and the proportions in which they are used are not intended as

restrictive but only as illustrating how a typical and especially desirable oil composition within the scope of my invention may be prepared. Repeated tests of novel oil compositions embodying my invention have established their effectiveness and value for the purposes in view.

What I claim is:

1. As a new article of manufacture, an oil composition comprising a solution of camphor in an oil consisting of a mixture of a lubricating oil with crude petroleum.
2. As a new article of manufacture, an oil composition comprising a solution of about  $\frac{1}{2}$  part of camphor in about  $15\frac{1}{2}$  parts of a mixture of crude petroleum and refined lubricating oil.
3. As a new article of manufacture, an oil

composition comprising a solution of about  $\frac{1}{2}$  part of camphor in about  $15\frac{1}{2}$  parts of a mixture comprising about  $11\frac{1}{2}$  parts of Pennsylvania or other paraffine base crude petroleum and about 4 parts of a medium motor lubricating oil.

4. As a new article of manufacture, an oil composition comprising a solution of camphor in mineral oil comprising both a mixture of refined lubricating oil and crude petroleum, the proportion of camphor not exceeding 2 ounces per pint of said composition.

In testimony whereof I hereunto affix my signature.

JOSEPH ALEXANDER X YOUNG.  
mark